

Patented Mar. 12, 1929.

1,705,298

UNITED STATES PATENT OFFICE.

KENNETH G. MACKENZIE, OF WESTPORT, CONNECTICUT, AND RAYMOND HASKELL, OF SUMMIT, NEW JERSEY, ASSIGNEES, BY MESNE ASSIGNMENTS, TO THE TEXAS COMPANY, OF NEW YORK, N. Y., A CORPORATION OF DELAWARE.

LUBRICATING OIL.

No Drawing.

Application filed August 21, 1924. Serial No. 733,283.

This invention relates to lubricating oils and more particularly to lubricating oils which are compounded, having hydrocarbon oils as a base.

5 In a certain type of automobile commonly in use having planetary transmission, the brake or transmission bands become worn and glazed so that when their surfaces are brought together in operation they do not 10 immediately grip but are caused to slip or "chatter". This is detrimental to the bands and produces uncertainty in the operation of the car.

In the endeavor to overcome such difficulties we have discovered that a small amount 15 of oxidized paraffine wax added to the usual hydrocarbon lubricating oil produces the very beneficial effect of preventing chattering.

20 The oxidized paraffine wax which is used in compounding our lubricating oil is produced by blowing crude or refined wax with air at an elevated temperature for a considerable period of time. A change takes place 25 in the chemical characteristics of the material, acidity developing not only as evidenced by the increasing acidity of the material itself, but also by the fact that some volatile acids may be condensed from the air 30 after it has passed through the hot material. In addition to these, however, certain saponifiable bodies or esters are formed, apparently from the condensation of acids and alcohols produced by the oxidation. These 35 esters are found to differ from the ordinary saponifiable oils or fats in that they do not readily saponify when treated with aqueous alkali solution but require treatment with an alcoholic solution of alkali to effect 40 complete saponification.

Upon separation of the constituents of the oxidized paraffine wax and compounding them separately with hydrocarbon lubricating oil, it is found that the previously mentioned esters when so used are particularly valuable for the prevention of chattering, even when added in quantities as small as 1/2 of 1%. We have also discovered that these same esters greatly increase the lubricating properties of a hydrocarbon oil. However, inasmuch as the acids and the unchanged wax in the oxidized material do not adversely effect the valuable properties of the esters, the oxidized wax itself may be

used for compounding, thus avoiding the expense involved in the extraction of the esters. 55

The following is a specific example of a method which has been found suitable in the oxidation of paraffine wax to produce a finished product having a sufficiently large proportion of esters. A charge of 50 pounds of paraffine wax is maintained at a temperature of from 295° to 300° F., in an enameled vessel while air is introduced in fine streams at the bottom of the vessel. The rate of introduction of the air is dependent upon the degree of distribution and contact which is obtained with the reaction materials. The oxidation is allowed to proceed for a period of about forty-eight hours, during 60 which time there is a loss of from 7 to 10 per cent in the weight of the charge due to volatilization products being carried off with the air stream. A typical sample of material produced by this treatment has the 65 following characteristics:

|                               |         |
|-------------------------------|---------|
| Acid number                   | 39.8    |
| Total saponification number   | 170.5   |
| Neutral saponification number | 130.7   |
| Melting point                 | 107°F.  |
| Neutral saponification number | 75 3.28 |

Acid number

|                                                                                                                                                                                                                                                |          |
|------------------------------------------------------------------------------------------------------------------------------------------------------------------------------------------------------------------------------------------------|----------|
| Another sample of the same material was treated first with alkali to neutralize the free acid and then treated with methyl ethyl ketone in which the paraffine wax is, for practical purposes, insoluble. The following results were obtained: | 85       |
| Free acid                                                                                                                                                                                                                                      | 22.4% 90 |
| Material insoluble in methyl ethyl ketone (unsaponifiable material, mainly wax)                                                                                                                                                                | 16.8     |
| Material soluble in methyl ethyl ketone (saponifiable material, mainly esters)                                                                                                                                                                 | 60.8     |

It will be observed from this data that the oxidized wax contains a large amount of saponifiable material and comparatively little unchanged wax. 100

To prepare a compounded lubricating oil having anti-chattering properties, oxidized wax is added while warm to hydrocarbon lubricating oil of proper quality in the proportion to give about 2% in the final product. Larger quantities of the oxidized wax may be used but we prefer to use very 105

small quantities since these have proven sufficient to give the desired results. The oxidized wax will mix without difficulty in the lubricating oil and will not separate out even at comparatively low temperatures.

While we have thus specifically described our invention, various modifications thereof may suggest themselves to those skilled in the art and we desire, therefore, to be limited only as indicated in the appended claims.

What we claim is:

1. A composition of matter comprising a hydrocarbon oil mixed with about 2% of 15 oxidized paraffine wax.
2. A composition of matter comprising a hydrocarbon oil and oxidized paraffine wax.
3. A composition of matter comprising a hydrocarbon oil mixed with a comparatively 20 small amount of oxidized paraffine wax.
4. A composition of matter comprising a hydrocarbon oil mixed with a comparatively small amount of paraffine wax which has been oxidized in such manner as to contain 25 a larger proportion of saponifiable material than of free acid.

5. A lubricating oil comprising a hydrocarbon oil and oxidized paraffin wax.

6. A lubricating oil comprising a hydrocarbon oil and a comparatively small 30 amount of neutral saponifiable material derived from the oxidation of paraffin wax.

7. A lubricating oil comprising a hydrocarbon oil and less than one per cent of neutral saponifiable material derived from the 35 oxidation of paraffin wax.

8. A composition of matter comprising a hydrocarbon oil mixed with a comparatively small amount of paraffine wax which has 40 been oxidized in such a manner as to contain a large proportion of saponifiable material.

9. A composition of matter comprising a hydrocarbon oil mixed with a comparatively small amount of oxidized paraffin wax whose content of saponifiable material and 45 free acid is in the proportion of greater than two to one.

In witness whereof we have hereunto set our hands this 15th day of August, 1924.

KENNETH G. MACKENZIE.  
RAYMOND HASKELL.